



The tensile tests were carried out with a Zwick apparatus at  $20^\circ \pm 1^\circ$  C. The breaking load (BL) and percentage elongation at break (El., percent) were determined.

These test pieces were aged in a ventilated oven for 5 days at  $105^\circ$  C.

The cables and test pieces corresponding to the following three comparative mixtures were prepared:

- (A) isoctyl phthalate containing 200 p.p.m. of hydrogenated bisphenol-A
- (B) isoctyl phthalate containing 200 p.p.m. of bisphenol-A, and
- (C) isoctyl phthalate not containing any stabilizer.

The following results were obtained:

#### ELECTRICAL PROPERTIES

|        | Kilometric resistance (MΩ) at 20° C. |                     |                    | Kilometric resistance (MΩ) at 60° C. |                     |                    |
|--------|--------------------------------------|---------------------|--------------------|--------------------------------------|---------------------|--------------------|
|        | Before ageing                        | Ageing after 5 days | Variation, percent | Before ageing                        | Ageing after 5 days | Variation, percent |
| A----- | 1,600                                | 1,500               | -6.5               | 25                                   | 20                  | -20                |
| B----- | 1,250                                | 550                 | -56                | 22                                   | 3.7                 | -82                |
| C----- | 1,200                                | 500                 | -58.5              | 19                                   | 3.5                 | -81.5              |

#### MECHANICAL PROPERTIES

|        | BL (kg./cm. <sup>2</sup> ) |                     |                    | El. (percent) |                     |                    |
|--------|----------------------------|---------------------|--------------------|---------------|---------------------|--------------------|
|        | Before ageing              | Ageing after 5 days | Variation, percent | Before ageing | Ageing after 5 days | Variation, percent |
| A----- | 256                        | 244                 | -4.5               | 318           | 302                 | -5                 |
| B----- | 246                        | 183                 | -25                | 336           | 178                 | -47                |
| C----- | 244                        | 185                 | -24                | 304           | 180                 | -40.5              |

These results show the distinctly higher resistance to ageing of mixture A containing the stabilizer according to the present invention.

#### EXAMPLE 2

The same composition as in Example 1 was used, except that isoctyl phthalate was replaced weight for weight by isodecyl phthalate. The operating conditions were similar. In Formula A, the isodecyl phthalate contained 200 p.p.m. of hydrogenated bisphenol-A; in Formula B, it contained 200 p.p.m. of bisphenol-A; in Formula C, it was used alone. The electrical and mechanical measurements, and ageing were carried out as in Example 1.

#### RESULTS

##### ELECTRICAL PROPERTIES

|        | Kilometric resistance (MΩ) at 20° C. |                     |                    | Kilometric resistance (MΩ) at 60° C. |                     |                    |
|--------|--------------------------------------|---------------------|--------------------|--------------------------------------|---------------------|--------------------|
|        | Before ageing                        | Ageing after 5 days | Variation, percent | Before ageing                        | Ageing after 5 days | Variation, percent |
| A----- | 1,900                                | 1,000               | -47.5              | 18                                   | 17.5                | -0.5               |
| B----- | 1,400                                | 275                 | -80.5              | 20                                   | 4.9                 | -75.5              |
| C----- | 1,300                                | 250                 | -80.5              | 15.5                                 | 4.1                 | -73.5              |

##### MECHANICAL PROPERTIES

|        | BL (kg./cm. <sup>2</sup> ) |                     |                    | El. (percent) |                     |                    |
|--------|----------------------------|---------------------|--------------------|---------------|---------------------|--------------------|
|        | Before ageing              | Ageing after 5 days | Variation, percent | Before ageing | Ageing after 5 days | Variation, percent |
| A----- | 264                        | 260                 | -1.5               | 349           | 324                 | -7                 |
| B----- | 268                        | 193                 | -26.5              | 346           | 190                 | -45                |
| C----- | 268                        | 201                 | -25                | 332           | 201                 | -39                |

#### EXAMPLE 3

The same composition as in Example 1 was used, except that "Alfol" 8-10 phthalate (trademark) was used as a plasticizer. "Alfols" are linear commercial alcohols obtained by the polymerization of ethylene. The operating conditions were similar. In Formula A, the "Alfol" 8-10

phthalate contained 200 p.p.m. of hydrogenated bisphenol-A; in Formula B, it was used alone. The electrical measurements and ageing were carried out as in Example 1.

#### RESULTS

|        | Kilometric resistance (MΩ) at 20° C. |                     |                    | Kilometric resistance (MΩ) at 60° C. |                     |                    |
|--------|--------------------------------------|---------------------|--------------------|--------------------------------------|---------------------|--------------------|
|        | Before ageing                        | Ageing after 5 days | Variation, percent | Before ageing                        | Ageing after 5 days | Variation, percent |
| A----- | 180                                  | 110                 | -39                | 4                                    | 2.7                 | -32.5              |
| B----- | 160                                  | 70                  | -56                | 3                                    | 0.7                 | -76.5              |

#### EXAMPLE 4

The procedure employed was similar to that of Example 3, but the "Alfol" 8-10 phthalate was treated beforehand with activated alumina, to purify same and improve its electrical properties. The same formulae were compared, A with 200 p.p.m. of hydrogenated bisphenol-A in the plasticizer and B without stabilization of the plasticizer. Electrical measurements and ageing were carried out as in Example 1.

#### RESULTS

|        | Kilometric resistance (MΩ) at 20° C. |                     |                    | Kilometric resistance (MΩ) at 60° C. |                     |                    |
|--------|--------------------------------------|---------------------|--------------------|--------------------------------------|---------------------|--------------------|
|        | Before ageing                        | Ageing after 5 days | Variation, percent | Before ageing                        | Ageing after 5 days | Variation, percent |
| A----- | 220                                  | 185                 | -16                | 8.8                                  | 5.5                 | -37.5              |
| B----- | 200                                  | 140                 | -30                | 4.9                                  | 2.1                 | -57                |

#### EXAMPLE 5

The same composition was used, except that 2-ethylhexyl phthalate was used as the plasticizer; the procedure followed was similar. In Formula A, the 2-ethylhexyl phthalate contained 200 p.p.m. of hydrogenated bisphenol-A; in Formula B it contained 200 p.p.m. of bisphenol-A; in Formula C, it was used alone. Electrical measurements and ageing were carried out as in Example 1.

#### RESULTS

|        | Kilometric resistance (MΩ) at 20° C. |                     |                    | Kilometric resistance (MΩ) at 60° C. |                     |                    |
|--------|--------------------------------------|---------------------|--------------------|--------------------------------------|---------------------|--------------------|
|        | Before ageing                        | Ageing after 5 days | Variation, percent | Before ageing                        | Ageing after 5 days | Variation, percent |
| A----- | 1,500                                | -----               | -----              | 10.5                                 | 6                   | -43                |
| B----- | 1,400                                | -----               | -----              | 8                                    | 5                   | -37.5              |
| C----- | 1,300                                | -----               | -----              | 6.5                                  | 5                   | -23                |

#### EXAMPLE 6

The following formulation was used:

| Parts                             |
|-----------------------------------|
| CPV ("Lucovyl" DS 1300) ----- 62  |
| 2-ethylhexyl sebacate ----- 16.5  |
| 2-ethylhexyl phthalate ----- 15.5 |
| Lead stabilizers ----- 3          |
| Fillers ----- 3.7                 |

In the first case (A) the 2-ethylhexyl sebacate and 2-ethylhexyl phthalate both contained 200 p.p.m. of hydrogenated bisphenol-A; in the second case (B), they contained 200 p.p.m. of bisphenol-A; in the third case (C), they contained 3% of trinonylphenyl phosphite. The procedure followed was similar to and the electrical

measurements and ageing were carried out as in Example 1.

## RESULTS

### ELECTRICAL PROPERTIES

|        | Kilometric resistance<br>(MΩ) at 20° C. |                           |                            | Kilometric resistance<br>(MΩ) at 60° C. |                           |                            |
|--------|-----------------------------------------|---------------------------|----------------------------|-----------------------------------------|---------------------------|----------------------------|
|        | Before<br>ageing                        | Ageing<br>after<br>5 days | Vari-<br>ation,<br>percent | Before<br>ageing                        | Ageing<br>after<br>5 days | Vari-<br>ation,<br>percent |
| A----- | 700                                     | 615                       | -12                        | 4.8                                     | 4.7                       | -2                         |
| B----- | 650                                     | 550                       | -15                        | 4.5                                     | 3.8                       | -15.5                      |
| C----- | 570                                     | 275                       | -51.5                      | 4.2                                     | 2.5                       | -40.5                      |

### EXAMPLE 7

Methylhexyldi - (4 - hydroxycyclohexyl)-methane was used in an amount of 200 p.p.m. in the plasticizer instead of hydrogenated bisphenol-A, according to the conditions set forth in Example 1. Increased resistance to ageing according to the evolution of the mechanical properties was observed.

### EXAMPLE 8

500 p.p.m., in relation to the plasticizer, of dimethyldi-(2,6-dimethyl-4-hydroxycyclohexyl)-methane were used instead of hydrogenated bisphenol-A, according to the conditions of Example 1, with a similar increase in the resistance to ageing.

What we claim is:

1. A stabilized resinous composition comprising (a) a chlorine-containing vinyl resin, (b) a biscyclohexanol of the formula:



wherein  $\text{R}_1$  and  $\text{R}_2$  are hydrogen or alkyl radicals containing from 1 to 18 atoms,  $\text{R}_3$  and  $\text{R}_4$  are hydrogen or alkyl radicals containing from 1 to 4 carbon atoms and  $m$  and  $n$  are integers from 1 to 4 and (c) at least one substance selected from the group consisting of tribasic lead sulfate, dibasic lead phthalate and dibasic lead phosphite.

2. A composition according to claim 1 in which the biscyclohexanol is isopropylidene-4,4'-biscyclohexanol.

3. A composition according to claim 1 in which the biscyclohexanol is isobutylidene-4,4'-biscyclohexanol.

4. A composition according to claim 1 in which the biscyclohexanol is methylhexyldi-(4-hydroxycyclohexyl)-methane.

5. A composition according to claim 1 in which the biscyclohexanol is hexyldi - (4 - hydroxycyclohexyl)-methane.

6. A composition according to claim 1 in which the biscyclohexanol is dimethyldi - (2,6-dimethyl-4-hydroxycyclohexyl)-methane.

7. A composition according to claim 1 in which the biscyclohexanol is di - (2,6-di-tert.-butyl-4-hydroxycyclohexyl)-methane.

8. A composition according to claim 1 in which the amount of the biscyclohexanol in the composition is from 20 to 20,000 parts per million based on the weight of the chlorine-containing vinyl resin.

9. A stabilizing composition for a chlorine-containing vinyl resin which comprises a biscyclohexanol of the formula:



wherein  $\text{R}_1$  and  $\text{R}_2$  are hydrogen or alkyl radicals containing from 1 to 18 carbon atoms,  $\text{R}_3$  and  $\text{R}_4$  are hydrogen or alkyl radicals containing from 1 to 4 carbon atoms and  $m$  and  $n$  are integers from 1 to 4 and at least one substance selected from the group consisting of tribasic lead sulfate, dibasic lead phthalate and dibasic lead phosphite.

10. A composition according to claim 9 in which the biscyclohexanol is isopropylidene-4,4'-biscyclohexanol.

11. A composition according to claim 9 in which the biscyclohexanol is isobutylidene-4,4'-biscyclohexanol.

12. A composition according to claim 9 in which the biscyclohexanol is methylhexyldi-(4-hydroxycyclohexyl)-methane.

13. A composition according to claim 9 in which the biscyclohexanol is hexyldi - (4 - hydroxycyclohexyl)-methane.

14. A composition according to claim 9 in which the biscyclohexanol is dimethyldi-(2,6-dimethyl-4-hydroxycyclohexyl)-methane.

15. A composition according to claim 9 in which the biscyclohexanol is di-(2,6-di-tert.-butyl-4-hydroxycyclohexyl)-methane.

### References Cited

#### UNITED STATES PATENTS

2,625,521 1/1953 Fischer et al. ----- 260—45.95

#### OTHER REFERENCES

Data Sheet published by National Lead Company, New York City, entitled "The Dutch Boy XL Series of Electrical Grade Stabilizers" received U.S. Patent Office Scientific Library July 12, 1965.

50 DONALD E. CZAJA, Primary Examiner

V. P. HOKE, Assistant Examiner

#### U.S. CL. X.R.

55 252—400, 407; 260—31.8, 45.95